

June 18, 1935.

S. P. MILLER

2,005,102

## DISTILLATION OF TAR

Filed May 21, 1931

5 Sheets-Sheet 1



**INVENTOR**

S. P. Miller

BY  
Fannie Davis, Kaufin & Edwards  
ATTORNEYS

June 18, 1935.

S. P. MILLER

2,005,102

DISTILLATION OF TAR

Filed May 21, 1931

5 Sheets-Sheet 2



June 18, 1935.

S. P. MILLER

2,005,102

DISTILLATION OF TAR

Filed May 21, 1931 5 Sheets-Sheet 3

Fig. 4.



Fig. 5.



Fig. 6.



INVENTOR

S. P. Miller

BY

Perris Davis, Koenig & Edwards

ATTORNEYS

June 18, 1935.

S. P. MILLER

2,005,102

## DISTILLATION OF TAR

Filed May 21, 1931

5 Sheets-Sheet 4

**INVENTOR**

S. P. Miller

BY

By  
Pennie Davis Hansen & Edwards  
ATTORNEYS

## ATTORNEYS

June 18, 1935.

S. P. MILLER

2,005,102

DISTILLATION OF TAR

Filed May 21, 1931

5 Sheets-Sheet 5

Fig. 8.



INVENTOR

S.P. Miller

BY

Pennia Davis, Martin & Adams

ATTORNEYS

## UNITED STATES PATENT OFFICE

2,005,102

## DISTILLATION OF TAR

Stuart Parmelee Miller, Englewood, N. J., assignor to The Barrett Company, New York, N. Y., a corporation of New Jersey

Application May 21, 1931, Serial No. 539,019

8 Claims. (Cl. 196—149)

This invention relates to new coal tar oils and pitches. These new products result from the distillation of coal tar in hot coal distillation gases and are formed by processes which prevent or minimize any substantial decomposition of the coal tar constituents. High yields of distillate are obtained and correspondingly low yields of pitch are produced. The products are substantially free from the decomposition products present in coal tar distillate and pitches produced by the ordinary distillation methods, particularly those produced on distillation at lower temperatures, and contain the less stable constituents which are decomposed by ordinary methods of distillation, and further these products contain ingredients present in the coal distillation gases employed for the distillation and these ingredients are recovered directly from the gases and incorporated in the products of the distillation. 10

The new coal tar oils contain higher boiling constituents of the coal tar which are relatively unstable and which are, therefore, decomposed by the usual methods of distillation. They contain oils originally present in vapor form in the coal distillation gases employed for the tar distillation. They are substantially free from pitch constituents. They are substantially free from decomposition products which result from the ordinary methods of distillation, particularly those produced at lower temperatures. The total distillate from a given coal tar represents a larger percentage of the constituents of the coal tar than is usually contained in total distillate and the oil fractions included in this invention comprise a correspondingly large percentage of distillate. The oils of this invention include distillate resulting from the production of pitch with a melting point of 260° F. and preferably 300° F. or greater and oil fractions including distillate of this range. They are suitable for use as creosote oil and for other uses to which ordinary coal tar distillate is put. 20

The pitches of this invention contain higher boiling constituents which are decomposed by ordinary distillation processes and are substantially free from decomposition products ordinarily present in coal tar pitches, particularly those produced by distillation processes in which materials are kept at distilling temperatures for a considerable period of time. They represent a lower percentage of the coal tar than does ordinary coal tar pitch. They include ingredients present in the coal distillation gases which are directly recovered during the tar distillation process and incorporated in the pitch produced. These directly recovered constituents include ingredients which are present in the coal distillation gases in the form of a fine suspension or mist known in the art as "tar fog". 30

The oils and pitches of this invention are produced by the distillation of tar in hot coal distillation gases such as hot coke oven gases or hot gas retort gases. They include pitches of the highest melting point and the maximum oil yield which can be obtained and pitches of lower melting point in the production of which an oil yield is obtained of lower percentage. They include pitches with a melting point of 260° F. or higher and the distillate corresponding to these pitches or fractions thereof or fractions of distillate which include oils of this range. 35

In producing the oils and pitches of this invention coal tar is brought into direct and intimate contact with hot coal distillation gases at or near their maximum temperature as they leave the ovens or retorts. The tar is atomized or sprayed into the hot gases with such volume, intensity and uniformity of spraying that the coke oven gases are immediately cooled from their maximum temperature to a materially lower temperature with simultaneous heating of the tar and repeated distillation thereof and with such thorough scrubbing of the hot gases as will free them from all or a greater part of their entrained carbon and pitch particles. The resulting admixed coke oven gases and vaporized oils are continuously withdrawn from the still while at a high temperature and subsequently cooled to condense the oils therefrom and the pitch produced is also continuously withdrawn from the still. 40

Coke oven gases, for example, leave the incandescent upper portions of the ovens at a temperature, for example, around 550 to 800° C. or higher, depending upon the construction of the ovens, the coking cycle, the degree of coking, etc. Such highly heated gases are at a temperature above that at which coking of pitch will occur but such coking is practically eliminated in the present process by subjecting the hot gases as soon as they enter the still to contact with an excessively large volume of spray of tar which is at a considerably lower temperature and which has adequate capacity for absorbing the heat of the gases as sensible heat and as latent heat. The effect of an excessive and intensive showering or spraying of tar into the gases is to suddenly and rapidly cool the gases to a temperature considerably lower than their initial temperature while at the same time rapidly but uniformly and in a controlled manner heating the tar and distilling vaporizable constituents therefrom. In this way the gases are rapidly cooled to a temperature such that objectionable coking can be readily avoided while the high temperature and heat content of the highly heated gases is nevertheless employed in a particularly advantageous manner for the rapid distillation of the tar. 45

The gases from horizontal gas retorts leave the retorts at temperatures of 500 to 700° C. or even much higher and are used to advantage for the 50

60

The gases from horizontal gas retorts leave the retorts at temperatures of 500 to 700° C. or even much higher and are used to advantage for the 60

distillation of tar by spraying the tar into the gases in the form of a fine intense spray and in sufficient volume to rapidly cool the gases and thus prevent excessive decomposition of the tar constituents.

The use of such highly heated gases has the further advantage that the gases even after being cooled by distillation of tar may still be at a high temperature, for example, when making 400° F. melting point pitch, around 350 to 400° C. and can be withdrawn from the still at such high temperatures with advantages which will herein-after be pointed out. The scrubbing of the highly heated gases is so effectively carried out that the gases themselves are thoroughly cleaned of entrained dust, pitchy material, etc., by the scrubbing operation and the distillate oils subsequently condensed from the gases are free or substantially so from such pitchy and other extraneous constituents, these constituents being scrubbed from the gases and added to the pitch residue.

The oils and pitches of this invention are obtained by the distillation of tars from various sources such as coke oven tars, gas retort tars, etc. Heavy tars or lighter tars or tarry oils can be distilled to produce the products of this invention. In the case of coke oven tar for example, the tar distilled may be the total tar produced at the coke oven plant or it may be the heavy tar separated in the collector main or the light tar or tarry oil separated in the condensers. The oil yield will not be the same in distilling a light tar as in distilling a total tar since there is more oil present in the former product. In other words, a light tar may be regarded as a total tar plus distillate oil and the oil yield will correspond to that from a total tar plus this additional amount of oil. In the claims the expression "obtainable by the distillation of a total tar" is not intended to limit the claims to products made by distilling only total tar but is intended to include the corresponding products made by other processes such as the distillation of a tarry oil.

The still in which the oils and pitches of this invention are produced includes means for introducing the hot coal distillation gases as well as means for introducing the tar and for withdrawing the pitch and also the admixed gases and vapors from the still. A total condenser or a series of fractional condensers is used for cooling the admixed gases and vapors to separate the coal tar oils therefrom. In order to take advantage of the maximum distillation capacity of the gases the still may be so located that the gases enter it at a temperature which is not greatly below that at which they leave the individual ovens or retorts. Any moderate drop in temperature of the gases can be compensated for by use of an added quantity of the heated gases. The volume and composition of the gases given off from adjacent coke ovens, for example, vary, the volume of the gases being greater at the beginning of the coking period after the oven is charged and being considerably less near the end of the coking period before the oven is pushed. Adjacent ovens are commonly charged at different times so that, for example, at the time one oven is charged the adjacent oven on one side will be well advanced in the coking period and the adjacent oven on the other side will also be well advanced but to a different extent. Accordingly by connecting gas off-takes from the individual ovens so that as the gases from these enter the still the variations in the amount, composition and temperature of the gases from any

particular oven with the progress of the coking cycle of that oven will be equalized with the gases coming from the other ovens and an approximately uniform volume of gases of approximately uniform average composition can be continuously obtained for the distillation.

In order to take full advantage of the high temperature and heat content of the superheated gases, for example, to obtain maximum distillation capacity and high melting point pitch, it is important to provide the still with heavy insulation and, as well as possible, avoid cooling of the gases after they leave the coke ovens and before they enter the still. Heat losses can be reduced to a minimum by providing the still and connecting pipes with heavy insulation.

The percentages of those ingredients present in the oils and pitches of this invention which are recovered directly from the coal distillation gases and incorporated in the oil and pitch produced are not uniform. Furthermore, they do not vary directly with the melting point of pitch produced or the boiling range of the oil obtained. The per cent of these ingredients directly recovered from the coal distillation gases depends upon the amount of tar distilled in a unit volume of the gases and the vapor and pitch content of these gases. The composition of coal distillation gases moreover varies with the nature of the coal distilled, the type of distillation apparatus employed and the temperature and rate at which the coal is distilled, etc.

The distilling capacity of a definite amount of the hot gases can be greatly increased, for example, by preheating the tar to remove water from the tar before it enters the still and for this purpose the tar may be heated to a temperature around but preferably somewhat higher than 100° C. The distillation capacity can be still further materially increased by preheating the tar to a higher temperature in order to supply from low temperature sources as much as possible of the latent and sensible heat required for distilling the oils of low and medium boiling points. For example in producing pitch with a melting point around 400° F. an increase in preheating of the tar from 100° C. to 200° C. before admitting it into the still resulted in an increased capacity of distillation per unit quantity of hot gas of about 40% to produce pitch of the same melting point and the distillation capacity of the gases per thousand cubic feet was increased from about 7.8 gallons of tar to about 10.8 gallons of tar. The following examples indicate the distillation capacity of hot gases with tar added at various temperatures. The tar when preheated to higher temperatures was preheated by the hot enriched gases leaving the still. The hot gases in each case entered at about 650° C. and the tar used contained about 2% water by volume. The distillation capacity is expressed as gallons of tar per thousand cubic feet of gas (the volume being calculated to standard conditions). Pitch of 400° F. melting point is made in each case:

| Tar temperature<br>° C. | Distillation capacity<br>Gallons |
|-------------------------|----------------------------------|
| 70                      | 7                                |
| 100                     | 7.5                              |
| 150                     | 9.4                              |
| 200                     | 11.7                             |
| 250                     | 16.3                             |

In actual operation it has been found that the per cent of tar constituents recovered directly

from the gases when expressed as per cent of the oil produced has varied at different plants. At one plant when the tar was heated to 200° C. and 400° F. melting point pitch was produced it was calculated that 4% of the oil obtained was recovered directly from the coal distillation gases and that 6.9% was recovered when the tar was preheated to 115° C. and 300° F. melting point pitch was produced. At another plant with a preheat of 177° C. when 400° F. melting point pitch was produced it was calculated that 6.6% of the oil was recovered directly from the gases and that 7.2% of the oil was recovered from the gases when 300° F. melting point pitch was produced and the tar was preheated at 88° C. At still another plant when the tar was preheated to 150° C. and 350° F. melting point pitch was produced it was calculated that 13.6% of the oil was recovered directly from the gases. Therefore although the oils and pitches of this invention contain constituents recovered directly from the gases, the percentage of the directly recovered constituents may vary over a considerable range within the scope of this invention.

As an illustration of the invention the products produced at one plant during a period of about a year's time may be mentioned. From two million gallons of coke oven tar nearly one and one-half million gallons of distillate oil were produced together with pitch having an average melting point of around 380° F. Oil yields from the coke oven tar distilled have been obtained of 75% or more over long periods of time with the production of pitch of melting point around 400° F. or higher. Pitch of 435° and 450° F. melting point has been made over considerable periods of time. The coke oven gases entering the still have been at a temperature around 550° C. or higher. The temperature of the gases and vapors leaving the still has varied for example between 350° and 400° C. When pitch of 300° F. melting point was produced with hot gases at about 550° C. the gases and vapors had an outlet temperature from the still of about 306° C. and the pitch left the still at a temperature of about 328° C., while with pitch of 400° F. melting point the gases and vapors left the still at a temperature of about 324° C. and the pitch left the still at a temperature of about 355° C. The still employed was about 20 feet long of rectangular cross section about 3½ feet wide and high and with six ovens connected by individual uptake pipes with the still.

It is important in producing the oils and pitches of this invention to provide for a rapid and intensive showering or spraying or atomizing of the tar into the hot gases so that the gases will be brought into immediate, continual and thorough contact with the spray and so that all parts of the still will be thoroughly flushed with liquid pitch and the walls kept clean from coke deposit. It is important that there shall be no local overheating of any portion of the still and that to avoid such overheating at all times there shall be in atomized form within the still a sufficient quantity of tar or partially distilled tar to absorb the heat of the hot gases by being itself distilled to pitch of the desired melting point under regulated conditions. It is important to avoid a deficiency of pitch or of partially distilled tar on any and all exposed surfaces of the distillation apparatus since such a deficiency would result in local over-distillation and the formation of coke because of the high temperature of the highly heated gases. Over-distillation and the forma-

tion of coke produce decomposition products, lower the oil yield and decompose constituents present in the tar which, so far as possible, are obtained in their original form in the oil and pitch products of this invention. Consequently in producing the oils and pitches of this invention all interior surfaces of the distillation apparatus should be continuously and intensively supplied and washed with the pitch or partially distilled tar. The same thorough and abundant scrubbing of the hot gases with the tar or partially distilled tar, which results in the cooling of the gases and the rapid distillation of the tar, also serves to keep all parts of the still surfaces flushed with partially distilled tar or pitch and prevents local overheating and coking thereon.

This thorough and abundant spraying of the gases with the tar or pitch may be accomplished by suitable mechanical devices of such a character and so located and operated that the tar or partially distilled tar will be projected into the hot gases and efficient subdivision of the tar accomplished. This is important not only to provide a large surface of evaporation and distillation but also to provide sufficient tar in the gas space of the still to absorb the heat of the hot gases therein, to keep the interior surfaces of the still flushed with the tar or partially distilled tar, to prevent objectionable coke formation and to adequately wash or scrub the gases to remove pitchy or carbon particles from them. One satisfactory means for atomizing the tar comprises a horizontal roll or a plurality of rolls or elongated cylinders rotating rapidly and with the cylindrical surface dipping into the tar or pitch at the bottom of the still and rotating at such a rate that it will spray the tar and pitch into the gas space of the still.

When tar is distilled to produce the oils and pitches of this invention and pitch of high melting point around 400° F. or higher is produced, the distillate includes heavy constituents which in an isolated state are solid or semisolid at ordinary temperatures. When the gases are cooled either directly or indirectly to condense all or most of the vapors therefrom in a single composite product the heavy constituents remain dissolved in the lighter oils and form with the lighter oils an oil suitable for creosote oil. The oils of this invention include oils of wide and also narrow boiling range suitable for creosote oil.

The total oil produced by the distillation of tar by a process yielding as much as 75% or more of the tar distilled, can be condensed as a single composite oil and employed for example as creosote oil or the admixed gases and vapors can be fractionally cooled and fractionally condensed and a plurality of oil fractions recovered. A sample of the oil produced at one plant showed a specific gravity at 38° C. of 1.110, only a trace of free carbon, and when subjected to distillation in accordance with the American Society for Testing Materials method No. D-246-28, showed up to 200° 1.1%, up to 210° 2.3%, up to 235° 8.3%, up to 270° 22.4%, up to 315° 34.3%, up to 355° 48.8% and the per cent of coke residue on the oil was 1.9%. It will be evident that the distillation can be carried out without the production of the maximum oil yield and the highest melting point pitch, and in this case an unusually high oil yield corresponding to the melting point of the pitch produced will be obtained.

Distilling coke oven tar, for example, in simple externally heated stills of 10,000 gallons ca-

5 capacity the oil yield is only around 44% when the distillation is carried to the point of producing pitch of around 300° F. and coking may begin before pitch of 400° F. melting point is reached.

10 5 With other methods of distillation somewhat higher yields of oils can be obtained to 300° F. melting point pitch but pitch as high as 400° F. has been made only with extreme difficulty. But by the process described new pitch products with a melting point of 400° F. are produced in a thoroughly successful manner and yields of around 15 75% or more of distillate are obtained from coke oven tar when distilled to the point of producing pitch of melting point of around 400° F. or higher; while with the production of pitch of lower melting point around 300° F. melting point it is possible to produce oil yields representing around 20 two-thirds or more of the tar distilled.

25 The invention will be further described in the accompanying drawings which show apparatus in which the oils and pitches of this invention may be produced by distillation in hot coal distillation gases. The drawings further illustrate in a graphic way the composition of the new oil products and pitches by representing the oil yield obtained on distillation to pitches of different melting points in producing the oils and pitches of this invention.

30 In the drawings Fig. 1 is a plan view of a coke oven battery equipped with a still for producing the oils and pitches of this invention.

Fig. 2 is an elevation partly in section of the still.

35 Fig. 3 is a cross section on the line 3—3 of Fig. 2.

Fig. 4 is an enlarged view partially in section showing one type of fractional condenser.

Fig. 5 is a section on the line 5—5 of Fig. 4.

Fig. 6 is a section on the line 6—6 of Fig. 4.

40 Fig. 7 is a diagrammatic view showing the still and the condensing system of Figs. 1-6.

Fig. 8 is a graph illustrating geometrically the relation of pitch melting point to oil yield of the new pitches and new oils obtained by the distillation of tar in hot coal distillation gases under the carefully regulated conditions by which either the new pitches or new oils of this invention are produced. The abscissæ represent percentage oil yields by volume based on the tar distilled and the ordinates represent pitch melting points in degrees Fahrenheit (air bath method).

55 In Figs. 1 to 3 part of a coke oven block or battery is indicated conventionally at 1 and part of the conventional by-product recovery system is illustrated. Individual coke ovens 2 have uptake pipes 3 leading to a collector main 4 common to a number of the ovens of the battery. The cross-over main 5 connects the collector main with the condenser 6 and the gas is then passed through the exhauster 7 to the ammonia absorber, the benzol scrubber, etc. Ordinarily ammonia liquor or ammonia liquor and tar are introduced into the collector main to cool the gases and keep the main flushed. A drain for the tar and ammonia liquor is indicated at 8 leading to the decanter 9 from which the tar is drawn off into the tar receptacle 10. Two condensers 6 are provided with means for drawing off the cooling liquids and light 60 tar into the decanter 11 from which the light tar collects in receptacle 12.

65 The apparatus thus far described which is illustrated only schematically varies somewhat in different coke oven plants and is described merely 70 for purposes of illustration.

75 A still 20 is located on the other side of the coke oven block. This still is of rectangular cross-section and is of such a length that four uptake pipes 21 pass upwardly into it from four individual ovens and two additional uptake pipes 22 connect adjacent ovens with the still. The internal uptake pipes 21 have lateral openings into the still and closures 23 operated by operating handles 24 for closing the individual uptake pipes during the charging of the coke ovens or 10 when it is desired to valve off any oven from the still. Clean-out openings 25 are provided for each of the uptake pipes.

15 The still and external pipes 22 are shown as provided with heavy insulation to prevent or reduce heat loss and reduction of temperature of the gases entering the still. If heavy insulation is provided the gases will enter the still at a temperature not materially below that at which they leave the individual ovens and they will thus 20 be available for distillation at their maximum temperature and in a highly heated condition.

25 The outlet for gases and vapors from the still is shown at 27 leading into an enlarged chamber 28 which serves as a settling chamber and which 25 may also serve as a distillation chamber for pre-heating and distilling tar as hereinafter described. A baffle 29 is located about the inlet to the chamber. The gas and vapor outlet 30 from the chamber 28 leads to a condenser 31 shown as 30 a three-stage fractional condenser from the bottom of which the cooled gases pass through the pipe 32 to the gas handling system for the coke oven plant.

35 The condenser illustrated is a three-stage condenser having two lower cooling sections 33 cooled by a suitable cooling liquid such as water and with an upper cooling section 34 which serves as a tar preheater and as a preliminary condenser for the gases and vapors. The upper tar 40 heating section has a tar supply pipe 35 leading to the tar coils 36 from which the preheated tar passes through the pipe 37 to the nozzle 38 located in the tower 28 between two packed sections 39 and 40 filled with broken up material 45 or cylindrical rings e. g. the well known Raschig rings. The upper section 39 serves to reduce entrainment of suspended particles while the lower section 40 serves the same purpose and in addition serves to bring the preheated tar into intimate contact with the admixed gases and vapors leaving the still. The preheated tar is thus partially distilled and the residue collects at the bottom of the tower 28 in the collecting section 41 and flows through the pipe 42 to one end of 50 the still 20.

55 At the other end of the still is located a pitch outlet shown as a trap 43 having an adjustable overflow outlet 46 leading to the trough 47 which is supplied with a rapidly moving stream of water through a supply pipe 44. The pitch is granulated by rapid chilling in the water in the trough which discharges the water and granulated pitch into the receptacle 45. This method of cooling and handling the pitch is only one of various methods which can be employed and for certain purposes the pitch can be cooled without admixture of water to give a solidified pitch product free from water.

60 Within the still 20 are located suitable atomizing or spraying devices for intensively atomizing or spraying the tar and pitch into the gases in such a way that all parts of the gases in the still are thoroughly scrubbed by the tar and pitch and so that all of the internal surfaces of the still 75

are intensively flushed by an excess of the tar or pitch. Where internal uptakes are employed the space back of these uptakes where the spray will not reach may be filled with suitable filling material. The mechanical spray devices shown are cylindrical rolls approximately 10" in diameter, three in number indicated at 48, 49 and 50 and driven at relatively high speed, for example 900 to 1,000 R. P. M. by motors 51 and 52 located at the ends of the still. The middle row 49 is coupled with one of the end rolls and is driven there-with by one of the motors, the coupling being shown at 53. In order to provide bearings 55 for the individual rolls part of the still is cut away as indicated at 54. The rolls are so located as to dip into the tar or pitch in the bottom of the still and the adjustable outlet for the pitch enables the depth to be regulated. By such regulation of the depth of the tar or pitch the extent to which the roll dips thereinto is governed and the character of the spray and the intensity may be governed at will by regulation of the depth of tar or pitch.

The production of the oils and pitches of this invention is not limited to processes which involve preheating the tar nor to processes involving the introduction of the tar into the gases and vapors escaping from the still to effect partial distillation before it enters the still but such pre-heating and partial distillation are advantageous and means for effecting them are shown in the drawings.

The condensing system shown is a fractional or multi-stage condensing system the first stage of which is a preheater for the tar in which the tar is preheated by indirect contact with the hot gases and vapors. The rate of distillation can be greatly increased by preheating the tar in this way while the gases are at the same time cooled to condense part of the distillate therefrom. The admixed gases and vapors are then further cooled in the lower stages of the condenser for example by indirect contact with cooling coils containing water. The cooling system shown in Figs. 4 to 7 has a water inlet 60 and a water outlet 61 supplying water to the lower cooling sections 33. Three outlets 62, 63 and 64 are provided for the condensate from the respective sections. Two return pipes 65 and 66 each leading to distributing nozzles 67 and 68 provide for returning the condensate from the upper section into the next lower section where it will blend with the condensate sprayed in such section. By returning the condensate from each of the two upper sections to the lower sections the condenser becomes a total condenser where all of the constituents are condensed and collected together to be drawn off through the bottom outlet 64. The construction of the condenser may vary and that shown in Figs. 4 to 6 is only one of various types of condensers which can be employed.

The tar supplied to the still may be the tar collected in the by-product system of the same plant and pumped from the tanks 10 and 12 by pumps 56 and 57 through pipe 58 to the still, or tar from another source of supply can be introduced through pipe 59.

The following data were collected when pitch of about 400° F. melting point was being produced in a still of the type shown in the drawings and these data may serve as an example of how the still is operated to produce the oils and pitches of this invention. Tar was supplied to the pre-heater at a temperature of around 63° C. and preheated by indirect contact with hot gases and

vapors to around 221° C. while the gases and vapors were cooled from around 293° C. to around 175° C. The tar preheated to 221° C. then entered the settling chamber where it was further heated and distilled by direct contact with the hot gases and vapors therein which were thereby cooled to a temperature of about 293° C. before they went to the preheater.

The intensive scrubbing to which the gases are subjected in the still during the distillation results in effectively cleaning the gases from suspended carbon and pitchy particles. As a result when the gases and vapors from the still are subjected to condensation, the oils condensed are clean oils substantially free from tarry or pitchy constituents and show only traces of so-called free carbon when subjected to the usual benzol extraction test.

In representing the production of the oils and pitches of this invention graphically in Fig. 8 the melting points of pitches in degrees Fahrenheit are plotted against the per cent of oil which distillation to that melting point yields. The oil is the oil actually distilled from the tar and the yield expressed does not include the oil recovered directly from the coal distillation gases. Those oils and pitches with a melting point above 260° F. which are produced by distillation in hot coal distillation gases by processes which yield distillate in excess of that expressed by the equation  $y=2.15x^2-246x+7290$  where  $y$  is the melting point of pitch in degrees Fahrenheit and  $x$  is the per cent of oil yield, are included in this invention and more particularly the invention includes only those oils and pitches so produced by processes where the ratio of oil yield to pitch is less than that expressed by the equation

$$y=.3125x^2-36.25x+1286,$$

and approximately that expressed by the equation  $30y=11x^2-1175x+38250$ . The graph of Fig. 8 shows all three of these curves and on this graph are also plotted the melting points and oil yields actually obtained for pitches as follows:

| Melting point | Oil yield |
|---------------|-----------|
| 400           | 76.3      |
| 400           | 82.5      |
| 400           | 79.0      |
| 400           | 81.4      |
| 355           | 73.4      |
| 300           | 71.7      |
| 360           | 66.7      |
| 350           | 67.6      |
| 325           | 68.6      |
| 310           | 62.8      |
| 295           | 62.8      |
| 260           | 60.1      |

My co-pending application Serial No. 326,769, filed December 18, 1928, of which this is in part a continuation, claims method and apparatus by which the oils and pitches of this invention may be produced. The curve  $30y=11x^2-1175x+38250$  of Fig. 8 includes the pitch of 400° F. melting point and oil yield of 75% described in that prior application and other oils and pitches the yield and melting point of which bear this relation to one another. The relation of the oil yield to the melting point of the pitch produced will vary and depends upon the composition of the tar treated, etc. The new products include the pitches and oils produced by processes in which the ratio of the oil yield to pitch melting point is as low as that represented by the curve  $y=2.15x^2-246x+7290$ , provided the pitch melting point is not below 260° F. and more particu-

larly those oils and pitches with a melting point not lower than 300° F., produced by the distillation of coke oven tar in hot coal distillation gases in which the ratio of pitch melting point to oil yield (based on the tar distilled) is included between the curves  $y=2.15x^2-246x+7290$  and  $y=.3125x^2-36.25x+1286$ .

The products of the present invention include a wide range of pitches and oils and pitches of various melting points as well as oils of various characteristics. The oils are clean oils substantially free from carbon or heavy pitch constituents and the term "clean" in the claims is used in this sense. Both the oils and pitches are substantially free from tar decomposition products, particularly those ordinarily produced by long-continued distillation, and contain constituents of coal tar ordinarily decomposed by the usual processes of distillation and in addition contain ingredients directly recovered from the coal distillation gases in which they are distilled.

In the claims "pitch melting point" refers to melting point in degrees Fahrenheit (air bath method, Journal of Industrial and Engineering Chemistry, vol. 10, pages 821, 822) and "oil yield" refers to percentage yield by volume based on net dry tar.

I claim:

1. Clean coal tar oils comprising oil condensed directly from coal distillation gases and a distillate oil, the distillate oil being obtainable by the distillation of a total coal tar to pitch with a melting point of at least 260° F. by a process according to which  $y$  equals between  $.3125x^2-36.25x+1286$  and  $2.15x^2-246x+7290$  where  $y$ =pitch melting point and  $x$ =oil yield, the upper limit of the boiling range of the oils condensed directly from the gases and the oils distilled from the tar being the same.

2. Clean coal tar oil fractions consisting of oil condensed directly from coal distillation gases and a distillate oil, the distillate oil being obtainable by the distillation of a total coke oven tar to pitch with a melting point of at least 260° F. by a process according to which  $y$  equals between  $.3125x^2-36.25x+1286$  and  $2.15x^2-246x+7290$  where  $y$ =pitch melting point and  $x$ =oil yield, the upper limit of the boiling range of the oils condensed directly from the gases and the oils distilled from the tar being the same.

3. Clean coal tar oil fractions consisting of oil condensed directly from coal distillation gases and a distillate oil, the distillate oil being obtainable by the distillation of a total coal tar to pitch with a melting point of at least 260° F. by a process according to which  $30y$  equals about  $11x^2-1175x+38250$  where  $y$ =pitch melting point and  $x$ =oil yield, the upper limit of the boiling range of the oils condensed directly from the gases and the oils distilled from the tar being the same.

4. Clean coal tar oil fractions consisting of oil

condensed directly from coal distillation gases and distillate obtainable by the distillation of a total coke oven tar to pitch with a melting point of at least 300° F., by a process according to which the ratio of the pitch melting point expressed as  $y$  and the oil yield expressed as  $x$  lies between

$y=2.15x^2-246x+7290$  and

$y=.3125x^2-36.25x+1286$ ,

the upper limit of the boiling range of the oils 10 condensed from the gases and the oils distilled from the tar being the same.

5. Pitch comprising pitch constituents recovered directly from coal distillation gases and pitch obtainable from the distillation of a total coal 15 tar to at least 260° F. melting point pitch by a process according to which  $y$  equals between

$.3125x^2-36.25x+1286$  and  $2.15x^2-246x+7290$

where  $y$ =pitch melting point and  $x$ =oil yield, the 20 boiling point of the lowest boiling of the constituents recovered directly from the gases and the lowest boiling of the constituents resulting from the distillation being the same.

6. Pitch comprising pitch constituents recovered directly from coal distillation gases and pitch obtainable by the distillation of a total coke oven 25 tar to pitch having a melting point of between about 260° F. and about 400° F. by a process according to which  $y$  equals between

$.3125x^2-36.25x+1286$  and  $2.15x^2-246x+7290$

where  $y$ =pitch melting point and  $x$ =oil yield, the boiling point of the lowest boiling of the constituents recovered directly from the gases and 35 the lowest boiling of the constituents resulting from the distillation being the same.

7. Pitch consisting of pitch constituents recovered directly from coal distillation gases and pitch obtainable by the distillation of a total coal tar 40 to pitch with a melting point of at least 260° F. by a process according to which  $30y$  equals about  $11x^2-1175x+38250$  where  $y$ =pitch melting point and  $x$ =oil yield, the boiling point of the lowest 45 boiling of the constituents recovered directly from the gases and the lowest boiling of the constituents resulting from the distillation of the tar being the same.

8. Pitch consisting of constituents recovered directly from coal distillation gases and constituents obtainable by the distillation of a total coke oven tar to pitch with a melting point of at least 300° F. by a process according to which the ratio of the pitch melting point expressed as  $y$  and the oil yield expressed as  $x$  lies between 55

$y=2.15x^2-246x+7290$  and

$y=.3125x^2-36.25x+1286$ ,

the boiling point of the lowest boiling of the constituents recovered directly from the gases and 60 the lowest boiling of the constituents resulting from the distillation of the tar being the same.

S. P. MILLER.